

## UNITED STATES PATENT OFFICE

2,475,129

METHOD OF SPINNING COLLAGEN  
SOLUTIONS

Arthur Cresswell, Stamford, Conn., assignor to  
American Cyanamid Company, New York, N.Y.,  
a corporation of Maine

No Drawing. Application January 14, 1949,  
Serial No. 71,047

2 Claims. (Cl. 18--54)

1

The present invention relates to the spinning of protein solutions and more particularly to an improved method of spinning collagen solutions.

In the spinning of filaments from protein material such as soy bean protein, gelatin, casein, collagen, albumen, keratin and the like, it is customary to make a solution or a suspension of the substance of the desired concentration, and jet the same under pressure through a multi-orifice spinnerette into a spin bath to cause solidification, coagulation or regeneration of the protein in a more or less oriented fibrous state, which filaments are then pulled away from the spinnerettes to form either a multi-filament or unitary strand as desired. Such spin baths usually include aqueous solutions of high concentrations of ammonium or metallic salts such as ammonium sulfate, zinc sulfate, magnesium sulfate and sodium sulfate.

In the spinning of such protein material, extreme difficulty has been experienced in starting the spinnerette due to the fact that in the starting up operation a quantity of the liquid to be spun leaks through the spinnerette and when it makes contact with the spin bath, covers the outer surfaces of the spinnerette and associated parts in a more or less tightly adherent film. Even though this film may be scraped or cleaned away, difficulty is experienced in that the coagulated or regenerated material tends to form again and clogs the holes of the spinnerette with the result that either the extrusion pressure is inadequate to open them or if they become unplugged, result in a broken filament.

An improved method of spinning collagen solutions has now been discovered which includes the following steps: preparing the collagen solution by dissolving collagen in an aqueous solution of an organic acid, removing fibers and other insolubles and extruding said solution through the orifices of a spinnerette, the spinnerette being coated with a basic nitrogen compound containing a long chain alkyl radical having more than 11 carbon atoms, into a spin bath containing an alkaline aqueous solution of a sulfate chosen from the group consisting of ammonium, sodium, zinc, magnesium and mixtures thereof, said coating being insoluble in and repellent of the spin bath solution.

Animal hides or skins are, by and large, the most readily available source of collagen. It is desirable in using this source of material, that unlimed hides be chosen. These may be fresh or green-salted calf skin, kip skin or other hides which are comparatively low in elastin content.

2

Kip skin is preferred because the collagen therefrom is of an optimum viscosity as compared to that of calf skin. These are fleshed and unhair down to the clean corium, which is that lamina- 5 tion of the animal hide containing the greatest proportion of collagen. If green-salted hides are used, the hides should be soaked before this treatment and also allowed to remain in the soaking liquid after cleaning until substantially salt free.

After cutting the corium into strips or small pieces for convenience in handling, the corium is covered with a dilute solution of an organic acid in the pH range of from 2 to 4. Any organic acid is satisfactory, although from 0.05 to 0.10 N formic acid or 0.5 to 1.0 N acetic acid are preferred. Any other concentration of other organic acids may be used so long as the pH of the solution falls within the specified range.

The corium is thus allowed to swell for from 16 20 to 24 hours in the acid solution at temperatures between 10° and 30° C. In this swelling, the hide imbibes from one to three times its own weight of liquid but by maintaining the temperature at this point below 30° C., gelatine-forming 25 conditions are definitely avoided.

Following the swelling, the excess liquid is drained off and the swollen corium mechanically disintegrated, for example, by a meat grinder, shredder or other form of sub-dividing mechanism which will break down the collagen fibers to the point where dissolution will be facilitated. In the mechanical disintegration step, heat may be developed due to friction and it is, therefore, important that the necessary steps be taken to 35 maintain the material during this operation at temperatures below 30° C.

At this stage and if the mechanical disintegration has been fine enough, practically all of the collagen will have gone into solution. Where this 40 collagen solution is highly concentrated, it will gel at 35° C. or below. Therefore, to separate the dissolved collagen from the insolubles, it is necessary to warm it slightly until fluidity has been reached. This will certainly be at a temperature 45 no higher than 60° C. While warming to this temperature, if mechanical agitation is carried on, any last traces of undissolved collagen will dissolve and the whole may then be centrifuged to remove elastin, hair fragments and other in- 50 soluble matter and then filtered as through cotton batting pads. The filtrate will be a clear heavily concentrated solution of collagen.

While the preferred source of collagen is the corium, as this involves handling a material of maximum collagen content with minimum in-

solubles, yet as a matter of fact, due to the distribution of collagen throughout the animal hide, it may be desirable to disintegrate the entire hide followed by collagen solution in dilute acid and the separation of the insolubles. Such a process while different in the last step due to the excessive amount of insolubles, does extract substantially all the collagen available.

The concentration of the collagen in its solution may be adjusted to a desired content appropriate for spinning, by the addition of a further amount of the dilute organic acid solution, such as that used for swelling and solution. It is preferred that the spinning solution contain from 5 to 15% collagen, although solutions of lower or higher collagen concentration may be used.

Strong salt solutions have been found satisfactory as coagulating baths, such as a 35% to saturated solution of ammonium sulfate with sufficient free ammonia to maintain a pH of 7.8 which is an isoelectric point of collagen. The free ammonia is useful for the purpose of neutralizing the organic acid introduced by the spinning solution. Another satisfactory bath is one containing 25% by weight of magnesium sulfate, buffered with triethanolamine to a pH of 7.8. Regardless of the particular coagulant used, it is highly desirable that the bath be maintained at from 20° to 30° C.

A considerable amount of experimentation has been carried on to provide a coating on spinnerettes which are usually composed of stainless steel, Monel metal, gold, platinum, palladium, rhodium, tantalum or alloys containing some or all of them, which will prevent the initial adhesion of the collagen material to the surface of the spinnerette. Substances found suitable in the spinning of viscose rayon filaments, such as lauryl pyridinium chloride and cetyl pyridinium chloride dissolved in the spinning bath were completely without effect in preventing initial adhesion of collagen material. Inasmuch as it appeared that greasy or waxy solids might have promise, a number of hydrocarbons such as paraffin, mineral oil and the like, were tried without success. Again, fatty acids such as stearic acid, palmitic acid and the like completely failed to overcome the difficulty. The higher alcohols, such as lauryl alcohol, the higher esters such as stearyl glyceride or palmytyl stearate completely failed to accomplish the desired purpose.

It was not until spin bath insoluble and repellent basic nitrogen compounds containing a long chain alkyl radical having twelve carbon atoms or more were tried that any sort of reasonable success occurred. These compounds, on the other hand, are outstanding in avoiding difficulties heretofore experienced in starting up operations with collagen material.

Where these compounds are heavy liquids, they may be applied as such or smeared over the outer surface of the spinnerettes and into the orifices therein. Where the substances are very viscous liquids, plastics or solids, they may be thinned or dissolved with organic solvents known as fat solvents such as volatile hydrocarbons such as benzene, gasoline and xylol and the chlorinated hydrocarbons such as chloroform, carbon tetrachloride or the like which may be readily volatilized.

Perhaps the most suitable class of materials for this purpose are the phosphatides of which lecithin is preferred. However, sphingomyelins and cephalines may also be used. Other materials eminently satisfactory are stearamide, ste-

arylamine, stearylguanidine, laurylamine, N,N-dimethyldodecylamine, 3-stearoxypropylamine, myristylamine, 6-octadecoxypyropylamine, N,N'-distearylalanyl amide, as well as the long chain alkyl cyanamides, dicyandiamides, melamines, guanamines, biguanides, guanylureas and the like where in all cases the alkyl radical has 12 or more carbon atoms.

Where the material is applied to the spinnerette in the form of a dilution or solution, chloroform and benzene are entirely satisfactory. It is preferred to make solutions containing from .01% to even as high as 25% in practice. It only becomes necessary to dip the spinnerette in a dilution or solution of the compound or to apply the same to the spinnerette either as a spray or with a brush and then cause the solvent to evaporate with the required amount of heat. Obviously the heat applied to cause evaporation of the solvent should be well below the melting point of the material used so as not to cause an abnormal flow which might clog the apertures. It has been found desirable during the solvent evaporation step to maintain a flow of gas such as air, nitrogen, carbon dioxide or the like through the spinnerette so as to keep the apertures from clogging with the coating material, while permitting the formation of a film thereon.

Such a treatment upon evaporation of the solvent deposits a very thin film on the spinnerette closely adherent to the surface thereof.

Such a coated spinnerette not only avoids the difficulty of the sticking thereto of collagen solutions or suspensions in the starting up operations but maintains the spinnerette in a perfectly free flowing state. It has been found, for instance, that a dilute organic acid solution of collagen containing from 5-15% of the latter may be satisfactorily extruded through a metal spinnerette as above when coated with a film of lecithin deposited from a chloroform solution thereof, immersed in an aqueous spin bath including ammonium sulfate from 35% to saturation and sufficient ammonia to maintain the pH of the bath at about 7.8, without initial sticking and for long periods of time without the production of imperfect filaments.

This application is a continuation in part of my copending application Serial No. 580,081, filed February 27, 1945.

While the invention has been described with particular reference to specific embodiments, it is to be understood that it is not to be limited thereto but is to be construed broadly and restricted solely by the scope of the appended claims.

I claim:

1. In a method of spinning collagen solutions prepared by dissolving collagen in an aqueous solution of an organic acid, removing fibers and other insolubles, the improvement which includes extruding the solution through the orifices of a spinnerette, the spinnerette being coated with a basic nitrogen compound containing a long chain alkyl radical having more than 11 carbon atoms, into a spin bath containing an alkaline aqueous solution of a sulfate chosen from the group consisting of ammonium, sodium, zinc, magnesium and mixtures thereof, said coating being insoluble in and repellent of the spin bath solution.

2. The method of claim 1 in which the spinnerette is coated with lecithin.

ARTHUR CRESSWELL.